

Oct. 20, 1931.

H. KURZ

1,828,325

PROCESS FOR THE MANUFACTURE OF RAILS WITH HARDENED HEADS

Filed July 7, 1928

Fig. 2.



Fig. 1.



Fig. 3.



Inventor:  
Heinrich Kurz  
by *John W. M.*  
Attorney

## UNITED STATES PATENT OFFICE

HEINRICH KURZ, OF DUISBURG-BUHRORT, GERMANY

## PROCESS FOR THE MANUFACTURE OF RAILS WITH HARDENED HEADS

Application filed July 7, 1928, Serial No. 291,036, and in Germany August 22, 1927.

When manufacturing rails with hardened heads and rolled articles of a similar kind, where certain areas or zones are to be improved, the following facts must be taken into consideration:

As is known carbon steel if suddenly chilled from a temperature above its critical temperature, shows hardness structures. The alteration of the properties of strength goes hand in hand with this alteration of structure, in such a manner that when the cooling is most pronounced, the greatest hardness and tensile strength occur simultaneously with diminished elongation. Between the extreme values of these martensite structures, and the pearlite structures occurring with slow cooling, with decreased hardness and tensile strength accompanied by increased elongation, there occur characteristic intermediate stages viz. "troostite", "osmondite" and "sorbite" whose elongation increases in the same sequence, whereas the hardness and the tensile strength fall.

The kinds of structures can be obtained:

(1) Either in such a manner that the rapidly chilled steel is by means of repeated heating subjected to an additional tempering up to the degree of improvement it is desired to obtain.

(2) In such a manner that by suitably regulating the time of cooling, the desired degree of hardening is obtained straight away.

The practical carrying out of these kinds of improvement is accompanied however, in the case of a rolled article of considerable length, as will be seen from the following, by great technical difficulties. It is of course economically more favorable if the heat still inherent in the rolled material after the rolling process, can be utilized for hardening purposes. If the improvement is effected according to the first of the two mentioned methods, then the material will have to be subjected to re-heating to quite definite degrees of temperature after the chilling. It is however very difficult to achieve a simple and effective attainment of these most favorable temperatures exactly.

Similarly with the second method difficulties are met with in regulating the cooling speed, as accurate and continuous control of temperature are required with this method, which is hardly practicable. But the greatest difficulty occurs in such cases where it is not desirable for manufacturing and technical reasons to harden the whole cross-sectional area. The brittleness in steel chilled in such manner is very great, so that in the case of 60 rails for instance, a hardening of the whole cross-sectional area of the rail head must be, for reasons of safety, avoided.

The invention relates in the first instance to a new process, preferably for treating 65 rails, where the running surface only is subjected to wear and tear, in such a manner that a greater degree of hardness and consequently a greater resistance to wear and tear is imparted to those parts. It becomes thus 70 possible to obtain in the work piece—the rail—the tenacity or toughness of the non-treated steel simultaneously with the hardness of the treated steel. Such a process possesses the advantage that the rails can 75 be rolled from material comparatively poor in carbon, which after being treated according to the present process, is superior to the usual carbon containing materials, both as regards tensile strength and resistance to 80 wear and tear. Thus the safety of railway working is appreciably improved.

In the case of the improved process, the finished rail on leaving the mill, moves as has already been similarly proposed, and 85 preferably after its end has been sawn off, slowly past nozzles, the liquid spray issuing from which effects a rapid chilling at the places to be hardened, for instance at the running surface of the head of the rail. The 90 quantity of liquid used depends on the sectional area of the rolled material on the depth of the desired hardening zone and on the temperature at which the rail leaves the rolls. It only requires a short sequence of 95 experiments to determine this quantity, for the case in point. The depth of the hardening can be regulated by the speed at which the rail passes the spray and by adjustment of the liquid supply. By this rapid chilling

at the places to be hardened a martensite structure is produced there, the heat remaining in the non-treated part of the cross-section flowing off to the chilled part, where it 6 may produce a tempering effect. Rails so hardened show as a rule a gradual transition from the hardness structure at the running surface to the normal non-treated ferrite-pearlite structure in the centre portion of the 10 head.

The invention provides that in such a process the rolled material is subjected to the cooling or the chilling treatment while lying down on the side, and that the part to be 15 especially subjected to the treatment is exposed to a substantially horizontal spray of the cooling medium. Thus it becomes possible to prevent the rail head to be treated from getting out of reach of the jets or 20 sprays of the cooling medium, even when a bend or twist occurs in the rail, which may be in various ways unsymmetrical in its cross section.

By reason of the laid down position of the 25 rail, the latter remains always in a horizontal position owing to its own weight, so that the horizontal spray of cooling medium impinges on the head everywhere and the head is consequently uniformly hardened.

30 In accordance with the invention also, the possibility of a bending or warping of the rail is further reduced by the fact that the rail foot, in addition to the head is subjected to chilling treatment so as to obtain an initial straightening. This cooling is effected at the same time that the head of the rail is chilled for hardening purposes. About two or three additional jets or sprays are, for 35 this purpose, provided opposite the chilling sprays for the head. This embodiment of the process is to be recommended when the head of the rail contains essentially more material than the foot. The cooling jets directed against the sole of the foot abstract a 40 certain amount of heat from it, with the consequence that the rail during the cooling can hardly, and certainly not to an inadmissible extent, bend or warp, and can in consequence be handled later on in an easier manner.

45 A further object of the invention, is to provide a modification of the process described, for the purpose of manufacturing hardened head-channel rails. The novelty consists therein, that the treatment of the running 50 surface of the rail is carried out by means of the cooling medium separately from the treatment of the check flange by the cooling medium. In this manner it is possible to fulfill the different conditions prevailing for 55 the hardening treatment both of the running surface and of the check flange, an advantage that may be of importance in the case of curved rails.

60 By maintaining constant high pressure of the cooling medium, the substantially hori-

zontal position of the cooling spray is ensured, whilst the place and the time of application of the treatment by the cooling medium as well as the depth of its action influencing the structure, is regulated by altering the quantity of the cooling medium as well as the speed at which the rail passes the sprays and the localization of the sprayed area of the work in relation to the path along which the rolled material has to travel.

An especial uniformity of hardening can be achieved in that any superfluous cooling medium which may possibly collect on the rolled material is removed from it by means of a current of some compressed medium, preferably air or steam directed on the top side of the web of the laid down rail by means of blow pipes grouped in the same manner as the hardening jets or nozzles.

An apparatus, suitable for carrying the new process into effect, and especially adaptable to the most varied cross-sectional shapes and dimensions in the rolled material, as well as to the most varied processes of hardening, is described hereinafter by way of example 85 90 95

These possibilities are created especially by reason of the fact that horizontal groups of hardening jets or sprays for the production of a substantially horizontal veil of the cooling medium are arranged alongside the path travelled by the material leaving the rolls. These groups of hardening jets or sprays are adapted to be brought into or out of their operative position separately. Further cooling nozzles or jets for the cooling medium are so arranged that the rolled material, when travelling past the above mentioned nozzles or jets is subjected to an additional cooling treatment of the sole of the rail foot.

100 By combining the various hardening jets or nozzles into groups that can be brought into or out of their operative positions individually, the operation of the process is greatly simplified, whereas by reason of the fact that said hardening jets or nozzles can be each separately regulated, opened or shut, the improved process has the necessary flexibility of regulation. This flexibility of regulation is further increased when the orientation of each single hardening nozzle or jet of a group can be separately set by swivelling said single jet in relation to the piping forming the other jet of said group.

110 A blast of air or steam under pressure is 120 directed against the top side of the web of the laid down rail through blow pipes, each of which is attached to a hardening spray.

115 The operation of the process according to the present invention is further greatly simplified by the fact that, on the one hand, the mechanism for controlling the supply of cooling medium to the hardening nozzles or jets is coupled to the mechanism for controlling the supply of the pressure medium (air 125 130

or steam) impinging on the top side of the web of the laid down rail, so as to provide a common control for both supplies, and, on the other hand, that a common control mechanism is provided for bringing simultaneously into or out of action all the hardening nozzles or jets forming a group and all the blow pipes for the pressure medium corresponding to said group.

10 In a corresponding manner it is finally possible to connect the mechanism for controlling the supply of cooling medium used for cooling the rail foot with the above first mentioned common control.

15 The accompanying drawings illustrate the invention and at the same time show an embodiment of apparatus for carrying the process into effect.

Figure 1 is an end view of said embodiment.

20 Figure 2 is a view similar to Figure 1, but in this case the hardening nozzles are shown in an inclined position which enables them to harden directly the check flange of a channel-head rail while the running surface of 25 the head of said rail is hardened only indirectly by convection.

Figure 3 is a front view of a separate hardening nozzle with an attached blow pipe.

25 After leaving the rolls (not shown) the rail is at a temperature of about 1100° C. and various types of known spraying means are placed adjacent the rolls to reduce the temperature of the rail so that the rail is not too hot for the subsequent hardening treatment. 35 The rail 10 is then passed in a longitudinal direction as to the length thereof over a hot bed 11 provided with a subjacent trough 12 or other suitable drainage means. A guide 13 is standing with respect to the hot bed 11 and abuts the rail 10 in its longitudinal travel.

40 The main supply of cooling medium passes through a longitudinal pipe 14 to a plurality of individually swinging spray groups arranged along the longitudinal path of the rail. Each hardening spray comprises two vertical branch-pipes 15 and 16 (Fig. 3), connected to a rotatable section of main supply pipe 14 corresponding to a group of hardening sprays and a nozzle 17 connected at the 45 lower ends of the vertical branch-pipes 15 and 16. Swivel flanges 18 and 19 are provided near the lower end of both branch-pipes 15 and 16, respectively, to allow adjustment of the orientation of each individual 50 spray against the particular part of the rail to be treated, according to requirements.

55 A blast of air or steam is conducted through blow pipes such as 20 arranged to rotate or swing with each spray and attached 60 to vertical pipe 15 by brackets such as 21. As many pipes 20 as there are nozzles 17 in a group are connected to a rotatable section of a supply pipe 22 corresponding in length with a rotatable section of the main supply pipe 14 and each of said pipes 20 is bent into

such a form that the blast of air or steam is directed against the upper side of the web of the lying down rail 10, when the nozzle 17 is brought in its operative position.

65 A plurality of stationary spray pipes 23, supplied by the main supply pipe 14, are positioned to direct jets of cooling medium against the sole of the foot of the rail 10 (to simplify the drawings only the lower end of 70 said spray pipes 23 are shown in Fig. 1). 75

80 Each branch-pipe 15, 16 is provided with a valve (not shown) independently of the fact that these branch-pipes are conjointly supplied by means of a common control. The mounting, individual regulating and common control arrangements for the various sprays and pipes may be such as are quite fully described in application Serial Number 370,699, divided from this present application and 85 filed June 13, 1929.

90 The raised position of the nozzle 17 and blow pipe 20, to clear the way when the rail is being removed sideways after the hardening treatment, is shown in dotted lines in Figure 1.

95 The quantities of cooling medium supplied through the sprays 17 and 23, and the quantity of blasting medium supplied through blow pipe 20, will depend on the characteristics required of the rail and the nature of the hardening treatment accordingly necessary.

100 Also the orientation of each spray nozzle 17, as effected by swivelling about the flanges 18 and 19 will be determined by the nature of the rail head and the particular part thereof to be treated.

105 What I claim and desire to secure by Letters Patent of the United States is:

1. A process for hardening the heads of rails by the action of a cooling medium which comprises passing the rail in a longitudinal direction and subjecting only the head thereof to the hardening treatment by means of a substantially horizontal spray of cooling medium.

110 2. A process for hardening the heads of rails by the action of a cooling medium which comprises conveying the rail in the direction of the length thereof, hardening only the top of the head of said rail by subjecting the same to a substantially horizontal spray of cooling medium while cooling the sole of the foot of said rail with an additional spray of said cooling medium thereby minimizing the tendency in the rail to bend due to the hardening treatment.

115 3. A process for hardening channel head rails by the action of a cooling medium which comprises conveying the rail in the direction of its length and hardening the running surface of said rail by subjecting the same to a substantially horizontal spray of cooling medium, the check flange of said rail being only 120 125 130

indirectly cooled and not hardened by the cooling medium.

4. A process for hardening channel head rails by the action of a cooling medium which comprises conveying the rail in the direction of its length, hardening the running surface of said rail by subjecting the same to a substantially horizontal spray of cooling medium, the check flange of said rail being free from direct impinging of said cooling medium and simultaneously cooling the sole of the foot of said rail with an additional spray of said cooling medium, thereby minimizing bending of the rail during the treatment.
5. A process for hardening the heads of rails by the action of a cooling medium which comprises conveying the rail in the direction of the length thereof, hardening only the top of the head of said rail by subjecting the same to a substantially horizontal high pressure spray of cooling medium and cooling the sole of the foot of said rail with an additional spray of said cooling medium, thereby minimizing the tendency in the rail to bend due to the hardening treatment.
6. A process for hardening the heads of rails by the action of a cooling medium which comprises conveying continuously the rail laid on its side in the direction of its length, hardening only a part of the head of said rail by subjecting said part to a substantially horizontal spray of cooling medium and varying the quantity and direction of said spray of cooling medium hardening a part of the rail head to vary the degree of hardening and the position of said hardened part, respectively.
7. A process for hardening the heads of rails by the action of a cooling medium which comprises conveying continuously the rail laid on its side in the direction of its length, hardening only a part of the head of said rail by subjecting said part to a substantially horizontal spray of cooling medium and subjecting laterally the rail to the cleaning action of a high pressure blasting medium.
8. A process for hardening channel head rails by the action of a cooling medium which comprises conveying the rail in the direction of its length, hardening the running surface of said rail by subjecting the same to a substantially horizontal spray of cooling medium, the check flange of said rail being free from direct impinging of said cooling medium, cooling the sole of the foot of said rail with an additional spray of cooling medium and subjecting the rail to a high pressure blasting medium to clean the surfaces of the rail.